

## UNITED STATES PATENT OFFICE

2,052,136

## STAINLESS FERROUS ALLOY

James P. Gill, Latrobe, Pa., assignor to Vanadium-Alloys Steel Company, Latrobe, Pa., a corporation of Pennsylvania

No Drawing. Application January 7, 1933,  
Serial No. 650,738

1 Claim. (Cl. 75—126)

This application is in part a continuation of my patent application Serial Number 495,423, filed November 13, 1930.

The purpose which I have in view is the improvement of stainless irons and steels by increasing their machinability.

Certain stainless steels are formed with a chromium content of from 8% to 20% and a carbon content of less than 1%, and with or without a content of less than 2% of nickel, tungsten and/or molybdenum, and with or without a content of less than 0.50% of silicon, manganese and/or phosphorus. However, these types of stainless steels are notoriously hard to machine and therefore their use for many industrial purposes, for which they are otherwise adapted, is restricted.

It is known that the addition of sulphur to steel increases machinability. Thus attempts have been made to improve such steels by the addition of a sulphur content under 0.15% together with a manganese content of approximately 1% and a phosphorus content of approximately 0.10%, but this results in the formation of manganese sulphide which renders the steel fibrous and thus impairs its physical qualities requisite for many uses.

Again, it has been proposed to add the sulphur in the form of zirconium sulphide or to add to the mix sulphur and zirconium, but the presence of zirconium renders the steel brittle, thus reducing its forgeability and impairing its physical properties.

In both the above instances the added metal, manganese or zirconium, has a greater affinity for the sulphur than has the chromium, and thus the ferrous alloy contains manganese sulphides or zirconium sulphides, and the chromium remains as chromium metal.

In my improved ferrous alloy, stainless iron or steel, the sulphur is combined with the chromium to form sulphides of chromium, either chromic or chromous sulphides or both, and I accomplish this result by adding the sulphur in the mix in the form of a sulphide of iron, ferrous sulphide or iron pyrite. The iron has less affinity for the sulphur than has chromium, and thus when the mix is melted the sulphur leaves the iron and combines with the chromium, the iron remaining as a necessary ingredient of the ferrous alloy and not as a deleterious intruder such as manganese or zirconium or not as introducing a new alloy in the mix as would be the case if copper matte were used as an ingredient. A certain percentage of manganese is present

in almost all steels, but I have discovered that a manganese content in excess of 0.25% will result in the formation of an appreciable amount of manganese sulphides which, as above explained, renders the steel fibrous and impairs its physical and stainless qualities.

By the use of my improved process I produce sulphides of chromium in the steel so that an ultimate analysis will show the product to contain up to 0.50% sulphur, the desirable range to obtain the improved properties being between 0.15% and 0.50%.

A heat of my improved steel, having an ultimate analysis of carbon 0.12%; chromium 12.75%; manganese 0.15%; silicon 0.30%; 15 phosphorus 0.13% and sulphur 0.23%, when annealed to a hardness approximating 190 Brinell can be machined approximately three times as rapidly as can steel of the same composition but lacking a similar percentage of the sulphur in the form of sulphides of chromium as an ingredient. Steel of this same heat, when quenched from a temperature of 1750° Fahr. and drawn to 1035° Fahr. disclosed the following physical qualities:—tensile strength 125000 pounds; yield 25 point 112000 pounds; reduction in area 62%; elongation in two inches 18.5%, and Brinell hardness 248.

It is obvious to those familiar with this branch of metallurgy that in my improved stainless ferrous alloy the sulphur is present as a sulphide of chromium. If it were present as a sulphide of iron the steel would not possess the high forgeability which it has been shown to possess. It is further obvious that with a manganese content of 0.25% or less the sulphur is not present in the form of manganese sulphide as the amount of manganese would be insufficient to absorb an appreciable amount of the considerable percentage of sulphur present.

Where zirconium is used as an ingredient the very purpose is to take up the sulphur and form zirconium sulphide.

The form in which the sulphur is present in stainless ferrous alloys is very important. If it be in the form of manganese sulphide, the corrosion-resisting qualities of the alloy are impaired and its structure is rendered fibrous. If it be in the form of zirconium sulphide the alloy is more brittle.

Both of these ingredients, manganese and zirconium are known to have a greater affinity for sulphur than has chromium, so it makes no difference in the ultimate result whether the sul-

40

35

45

50

55

phur and the manganese or the zirconium are added separately or in the form of sulphides.

Again the machining qualities of my improved ferrous alloy are far superior at any hardness than those at the same hardness of a corresponding steel not having as a constituent sulphides of chromium within the limits above set forth.

The use of sulphide of chromium as a constituent of my steel does not appreciably decrease the resistance of the steel to staining or corrosion, and samples tested under the standard salt spray test show my steel to have substantially the same corrosion resistance as do similar steels which lack the sulphide of chromium content.

The physical qualities of my improved stainless steel may be further improved by the addition of not more than 2% of nickel.

I claim:—

A stainless ferrous alloy having improved machinability without substantially impaired forgeability and consisting essentially of carbon from .05% to .50%; chromium from 8% to 20%; silicon from .10% to .50%; manganese from .05% to .25%; phosphorus from a trace to .04%; sulphur from .15% to .50%, the major portion of the sulphur being present in the form of a sulphide of chromium, and the balance of the alloy consisting of iron.

JAMES P. GILL. 15